

# United States Patent

[11] 3,563,299

[72] Inventor **Manfred Schrage**  
Dudenhofen near Offenbach, Germany  
[21] Appl. No. **679,684**  
[22] Filed **Nov. 1, 1967**  
[45] Patented **Feb. 16, 1971**  
[73] Assignee **Messer Griesheim, GmbH**  
Frankfurt am Main, Germany  
a corporation of Germany  
[32] Priority **Nov. 12, 1966**  
[33] Germany  
[31] **M 71642**

[54] **PROCESS FOR THE WASHING AND PURIFYING OF MOLTEN METALS**  
6 Claims, 2 Drawing Figs.  
[52] **U.S. Cl.** ..... 164/82,  
164/55, 164/66  
[51] **Int. Cl.** ..... B22d 11/00  
[50] **Field of Search** ..... 164/66,  
259, 82, 306, 307, 55—57, 283, 281, 134; 266/37

[56]

## References Cited

### UNITED STATES PATENTS

|           |         |                        |         |
|-----------|---------|------------------------|---------|
| 3,395,750 | 10/1968 | Keene .....            | 164/259 |
| 3,300,824 | 1/1967  | Ross .....             | 164/66  |
| 2,889,596 | 6/1959  | Savage et al. ....     | 164/283 |
| 3,224,051 | 12/1965 | Brown, Jr. et al. .... | 164/66  |
| 963,973   | 7/1910  | Wright.                |         |
| 3,411,566 | 11/1968 | Astrov et al. ....     | 164/55X |
| 3,392,009 | 7/1968  | Holmes et al. ....     | 164/66X |

### FOREIGN PATENTS

1,031,317 6/1966 Great Britain.

*Primary Examiner*—Charles W. Lanham

*Assistant Examiner*—V. K. Rising

*Attorney*—Connolly & Hutz

**ABSTRACT:** A process for washing and purifying molten metals in continuous casting operations includes injecting a flash gas on the molten surface of the continuously moving workpiece in such a manner that the drawn off gases prevent the admission of air.



PATENTED FEB 16 1971

3,563,299

Fig. 1



Fig. 2



## PROCESS FOR THE WASHING AND PURIFYING OF MOLTEN METALS

### BACKGROUND OF THE INVENTION

The invention relates to a process for the washing and purifying of molten metals with respect to continuous casting processes by the injection of gases or gas mixtures.

It is known to treat molten metal by injecting gases, for instance by injecting oxygen in refining or by injecting argon on melts located in the casting ladle for decontamination purposes. Furthermore, it is customary during the pouring into the cast iron mold in continuous casting installations to protect the melt surface and the casting current against air admission by means of an argon screen or mist.

The utilization of both processes has the disadvantage that they must be undertaken separately, in two steps, i.e. in the casting ladle and in the continuous casting mold, if the decontamination effect is not to be lost during pouring.

### SUMMARY OF INVENTION

The object of the invention is to eliminate the above disadvantages and to provide a process which combines an effective washing of the liquid metal with an effective casting protection.

In accordance with this invention the flash gas is blown on the molten surface of the continuously moving work piece in such a manner that the drawing off gases effect a casting protection against air admission. A lance may be suitably used for the injection of the flash gas.

The desired exchange of material takes place at the contact surfaces between gas and melt. The gas rising from the melt surface simultaneously protects the melt surface and casting current. A considerable advantage of this process lies particularly in that the melt can be very effectively decontaminated by the continuously renewing surfaces which form in the cast-iron mold.

An arrangement for the carrying out the inventive process in an advantageous manner, includes a lance for the injection of the flash gas between the distribution groove or casting ladle for the molten substance and the cast-iron mold. Between the distribution groove or ladle and the cast-iron mold, a box or bellows like protective device can also be arranged for obstructing or baffling the gases drawn off through an outlet. The protective device can be placed under more or less intensely reduced pressure, to assure that the gases rising from the melt surface are drawn off. In this simple and advantageous manner the decontaminating reaction is simultaneously intensified by the combination of flash gas process and reduced pressure.

In the inventive process the inert or reactive flash gas can be utilized as a carrier for gaseous, liquid or solid additives.

### THE DRAWINGS

FIG. 1 shows a distribution groove with cast-iron mold and lance; and

FIG. 2 shows an arrangement according to FIG. 1 with a protective device.

### DETAILED DESCRIPTION

As shown in FIG. 1 the melt passes from the distribution groove or ladle 1 of the continuous casting installation to the cast-iron mold 2 together with the continuously moving work-piece 3. The flash gas is blown on the surface of the melt, disposed in the cast-iron mold 2, through lance 4 of any desired construction. The desired transfer of material between melt and gas takes place in the contact zone 5. The rising gases protect both the melt surface as well as the casting current and prevent the admission of air by thereby acting as a shield.

The space between distribution groove 1 and cast-iron mold

2 can, according to FIG. 2, be further surrounded by a box or bellowslike protective device 6, so that the gases drawn off through an opening 7 located in this box, are first baffled to enhance the casting protection.

5 Furthermore, reduced pressure can be provided at the discharge opening 7 of the casting protection device, so that the drawn off gases are speedily drawn off and so that the decontamination reaction is accelerated by the combination of the reduced pressure and blowing.

10 The invention is, of course, in no way limited to the embodiments described above and illustrated in the drawing, since various modifications are possible without deviating from the scope of the invention. Thus, flash gas, for example, can be utilized as a carrier for certain solid, liquid or gaseous additives.

15 I claim:

1. In a process for flushing, purifying and degassing molten metal with a gas stream in a continuous casting installation including a casting ladle for the molten metal and there being

20 beneath said casting ladle a cast-iron mold for continuously forming a workpiece, comprising directing the gas stream into the surface of the molten metal in said mold below said ladle, penetrating the gas stream into the molten metal a depth for flushing, purifying and degassing the same while the casting

25 operation is taking place, drawing off the gas from the molten metal while the casting operation is taking place, creating a shield with the drawn-off gas to prevent the admission of air to the surface of the molten metal, the gas being directed by a lance between the ladle for the molten substance and the cast-iron mold, baffling the drawn off gas by means of a protective device disposed between the ladle and cast-iron mold and said device having a gas outlet therein, and maintaining said device under reduced pressure.

30 2. In a process as set forth in claim 1 wherein the gas is used as an additive carrier.

3. A process for flushing, purifying and degassing molten metal with a gas stream in a continuous casting installation including a casting ladle for the molten metal and there being

40 beneath said casting ladle a cast-iron mold for continuously forming a workpiece, comprising directing the gas stream into the surface of the molten metal in said mold below said ladle, penetrating the gas stream into the molten metal a depth for flushing, purifying and degassing the same while the casting operation is taking place, applying mechanical means for drawing off the gas from the molten metal while the casting operation is taking place, and creating a shield with the drawn-off gas to prevent the admission of air to the surface of the molten metal.

45 4. In a process as set forth in claim 3 including baffling the drawn off gas by means of a protective device disposed between the ladle and cast-iron mold and said device having a gas outlet therein.

5. A process for flushing, purifying and degassing molten metal with a gas stream in a continuous casting installation including a casting ladle for the molten metal and there being

55 beneath said casting ladle a cast-iron mold for continuously forming a workpiece, comprising directing the gas stream into the surface of the molten metal in said mold below said ladle, penetrating the gas stream into the molten metal a depth for flushing, purifying and degassing the same while the casting operation is taking place, drawing off the gas from the molten metal while the casting operating is taking place, creating a shield with the drawn-off gas to prevent the admission of air to the surface of the molten metal, providing a bellows formation

60 between the ladle and mold with the drawn-off flowing out of the bellows formation, and utilizing the bellows formation to baffle the drawn-off gas flowing therefrom.

65 6. In the process as set forth in claim 5 including applying mechanical means to the bellows formation for drawing off the gas from the molten metal.